

## UNITED STATES PATENT OFFICE

2,112,864

PROCESS FOR PRODUCING FAST DYEINGS  
ON THE FIBER

Enrico Pool and Gérald Bonhôte, Basel, and Carl Apotheker, Riehen, near Basel, Switzerland, assignors to firm of Society of Chemical Industry in Basle, Basel, Switzerland

No Drawing. Application January 19, 1935, Serial No. 2,602. In Switzerland January 27, 1934

14 Claims. (Cl. 8—5)

Various processes are known for the production of topical dyeings on the fiber by making thereon insoluble azo-dyestuffs. Very good results are obtained, for example, by grounding the whole fabric with the coupling component and applying the diazo-compound only at certain places, or by printing locally with mixture of coupling component and anti-diazo-compound or diazo-amino-compound and then forming the azo-dye-  
5 stuff by a suitable treatment. All these processes have the common feature that the diazo-compound or the product which contains the diazo-compound ready made, such as the anti-diazotate or the diazo-amino-compound, is produced by  
10 treatment of the diazotizable base with nitrous acid not on the fiber but in a separate operation, in absence of the coupling component. It has not been possible hitherto, without an essential impoverishment of the result in respect of depth  
15 and beauty of the coloring, to simplify the production of topical dyeings of azo-dyestuffs on the fiber by printing diazo-component and coupling component together on the fiber and then forming the dyestuff by causing nitrous acid to act on  
20 the mixture of coupling component or diazo-component.

The present invention relates to a process in which the mixture consisting of a suitable (of not too low a melting point and little volatile) diazotizable amine, and alkali salt of a coupling component or a mixture of a coupling component and caustic alkali, and alkali nitrite is applied to the fiber and then, by passage of the fiber through acid, while avoiding high temperature (preferably  
30 at a temperature that does not exceed 25° C.), the amine is first diazotized and then, by a passage through an acid binding agent as a second operation the coupling is produced; in this manner dyeings are obtained which are incom-  
35 parably finer than those obtainable by the hitherto known methods on the fiber by diazotization of the diazo-component in the presence of the coupling component, and are equal not only to the dyeings obtained with the aid of prepara-  
40 tions of diazo-amino-compounds or of nitroso-amine, but also to those obtained by direct printing of the diazo-compound on the goods prepared with the coupling component. In many cases it may be of advantage, for the purpose of  
45 obtaining pure coloring, to add formaldehyde to the printing color. The invention owing to the simplicity of the process involves an important technical advance and could not be predicted from the available literature.

50 Among diazotizable amines having not too low

a melting point are included such amines which do not melt much below 60° C. A great number of such bases is illustrated in the examples to follow. Among the diazotizing bases which come into consideration for the new process those are particularly useful which contain two aromatic nuclei linked by bridges, such as diaryl ethers, azo-compounds, monoacyl derivatives of aromatic diamines containing in the acyl radical an aromatic nucleus. Among the coupling components the arylides of hydroxycarboxylic acid are particularly valuable, and among these again the 2:3-hydroxynaphthoic acid and the 2:3-hydroxyanthracene-carboxylic acid.

The production of the dyeings in accordance with the invention may be combined with the production of other dyestuffs, for example with that of aniline black, or effects produced by vat-dyestuffs or their leuco-sulfuric acid esters or the like.

20 The following examples illustrate the invention:—

## Example 1

A mixture is made from 331.2 parts by weight of 4-(1'-methyl)-phenoxyacetylarnino-2:5-dimethoxy-1-aminobenzene, 232.2 parts of 2:3-hydroxynaphthoic acid-3'-nitranilide, 186 parts of sodium nitrite, 2 parts of sodium hydroxide and 69.1 parts of crystallized sodium acetate or the corresponding quantity of the anhydrous product. From this mixture there is prepared a finely subdivided printing color by carefully making a paste of 8 grams of the mixture, 38 cc. of water, 3 cc. of sodium hydroxide solution of 34° Bé., 3 cc. of Turkey red oil, 5 cc. of glycerin and 43 grams of neutral starch tragacanth thickening. The fabric is printed with this printing color, dried and quickly passed through an aqueous hydrochloric acid solution of 2 per cent. strength, containing 50 grams of sodium chloride per liter. The fabric is then wrung out and treated with an aqueous sodium carbonate, sodium bicarbonate or sodium acetate solution of 3—5 per cent. strength for a short time, whereby there is very quickly developed a fast, deep, pure violet color. The fabric is then rinsed and treated in a soap bath at the boil.

## Example 2

A mixture is made from 240.1 parts by weight of benzene-azo-ortho-anisidine, 288.9 parts of 2:3-hydroxynaphthoic acid-4'-methoxyanilide, 245 parts of sodium nitrite, 24.2 parts of crystallized sodium acetate and 2 parts of sodium hy-

50

55

## Example 5

A printing color is prepared from 6 grams of  $\beta$ -naphthol, 6.5 grams of 4-amino-3:2'-dimethylazobenzene, 2.5 grams of sodium nitrite, 5 cc. of sodium hydroxide solution of 34° Bé., 5 cc. of Turkey red oil, 5 cc. of glycerine, 35 cc. of water and 37 grams of neutral starch tragacanth thickening. The goods are printed with this finely subdivided printing color, dried and then rapidly passed through an aqueous solution containing per liter 50 grams of sulfuric acid and 200 grams of Glauber's salt. The goods are now wrung out, hung in the air for a minute and treated at 60–70° C. with a sodium bicarbonate solution of 4 per cent. strength. Rinsing and soaping follow. There is obtained a Bordeaux red dyeing.

## Example 6

273 parts by weight of 4:4'-dichloro-2-amino-1:1'-diphenylether are mixed with 264.3 parts of 2:3-hydroxynaphthoic acid-2'-methoxyanilide, 222 parts of sodium nitrite, 2 parts of sodium hydroxide and 38.3 parts of crystallized sodium acetate. The printing color is made as follows:—

8 grams of the above mixture are very finely suspended in 3 cc. of sodium hydroxide solution of 34° Bé., 3 cc. of Turkey red oil, 37 cc. of water, 5 cc. of glycerine, 2 cc. of formaldehyde solution of 40 per cent. strength and 42 grams of neutral starch tragacanth thickening. The further procedure is as described in Example 1, but during the drying too high a temperature should preferably be avoided. There is obtained a pure red dyeing.

## Example 7

294 parts of the ethyl ester of 2-amino-4'-chloro-1:1'-diphenylether-4-carboxylic acid are well mixed with 246 parts of 2:3-hydroxynaphthoic acid-2'-methoxyanilide, 208 parts of sodium nitrite, 2 parts of sodium hydroxide and 50 parts of crystallized sodium acetate.

8 grams of this mixture are very finely suspended in 3 cc. of sodium hydroxide solution of 34° Bé., 3 cc. of Turkey red oil, 37 cc. of water, 5 cc. of glycerine, 2 cc. of formaldehyde solution of 40 per cent. strength and 42 grams of neutral starch tragacanth thickening. Further procedure is as described in Example 1, drying at too high a temperature being preferably avoided. There is obtained a pure red dyeing.

The following table shows a number of other dyeings which can be produced in accordance with this invention:—

| 60 | Diazo-component                                                                                                                                                                                                                                                                                                                                                                                                                                  | Coupling-component                                                                                                                                                                                                                                  | Color of the combination produced on cotton                             | 60 |
|----|--------------------------------------------------------------------------------------------------------------------------------------------------------------------------------------------------------------------------------------------------------------------------------------------------------------------------------------------------------------------------------------------------------------------------------------------------|-----------------------------------------------------------------------------------------------------------------------------------------------------------------------------------------------------------------------------------------------------|-------------------------------------------------------------------------|----|
| 65 | 4:4'-dichloro-2-amino-1:1'-diphenylether<br>2-amino-1-methyl-4-nitrobenzene<br>1-amino-2-methyl-4-nitrobenzene<br>4-amino-3:2'-dimethyl-azobenzene<br>1-amino-2-methoxy-5-chloro-4-benzoylaminobenzene<br>1-amino-2-methoxy-5-methyl-4-benzoylaminobenzene<br>1-amino-2:5-diethoxy-4-benzoylaminobenzene<br>Para-chlorophenyl-azo-cresidine<br>o-anisol-azo- $\alpha$ -naphthylamine<br>1-amino-2-methyl-4-nitrobenzene                          | Di-(acetic acid)-ortho-ortho'-tolidine<br>2:3-hydroxynaphthoic acid-anilide<br>2:3-hydroxynaphthoic acid-2'-methylanilide<br>2:3-hydroxynaphthoic acid-anilide<br>2:3-hydroxynaphthoic acid-4'-methoxy-anilide<br>2:3-hydroxynaphthoic acid-anilide | Yellow.<br>Scarlet.<br>Blue red.<br>Bordeaux.<br>Red violet.<br>Violet. | 65 |
| 70 | 2:3-hydroxynaphthoic acid-anilide<br>3-hydroxy-1:2-benzofluorenone<br>2:3-hydroxynaphthoic acid-anilide<br>2:3-hydroxycarbazole-carboxylic acid-parachlor-anilide<br>2:3-hydroxynaphthoic acid-4'-ethoxy-anilide<br>2:3-hydroxynaphthoic acid-4'-methoxy-anilide<br>2:3-hydroxynaphthoic acid-1'-naphthylamide<br>2:3-hydroxynaphthoic acid-anilide<br>2:3-hydroxynaphthoic acid-2'-methoxyanilide<br>2:3-hydroxynaphthoic acid-2'-naphthylamide | Blue.<br>Black.<br>Violet black.<br>Brown.<br>Scarlet.<br>Red.<br>Red.<br>Blue.<br>Garnet.<br>Black.                                                                                                                                                | 70                                                                      |    |

| 5  | Diazo-component                                      | Coupling-component                                                               | Color of the combination produced on cotton | 5  |
|----|------------------------------------------------------|----------------------------------------------------------------------------------|---------------------------------------------|----|
| 5  | $\alpha$ -naphthylamine                              | 2:3-hydroxynaphthoic acid-1'-naphthylamide                                       | Bordeaux.                                   |    |
|    | 2-amino-5-acetyl-amino-4:4'-dichloro-diphenylether   | 2:3-hydroxynaphthoic acid-4'-ethoxy-anilide                                      | Bordeaux red.                               |    |
|    | 2-amino-4-aceto-4:4'-dichloro-diphenylether          | 2:3-hydroxynaphthoic acid-2'-methoxy-anilide                                     | Red.                                        |    |
|    | 2-amino-5-acetyl-amino-4:4'-dimethoxy-diphenyl-ether | 2:3-hydroxynaphthoic acid-4'-methoxy-anilide                                     | Violet.                                     |    |
| 10 | Aminoazobenzene                                      | 2:3-hydroxynaphthoic acid-anilide                                                | Bordeaux.                                   |    |
|    | 4-amino-2':3-dimethyl-azobenzene                     | 2:3-hydroxynaphthoic acid-3'-nitro-anilide                                       | Garnet.                                     | 10 |
|    | 1-amino-2:5-dimethoxy-4-benzoylaminobenzene          | 2:3-hydroxynaphthoic acid-anilide                                                | Blue.                                       |    |
|    | 1-amino-2-chloro-5-methoxy-4-benzoylaminobenzene     | 2:3-hydroxynaphthoic acid-2'-methoxy-anilide                                     | currant.                                    |    |
|    | 4:4'-dichloro-2-amino-diphenylether                  | 2:3-hydroxycarbazole carboxylic acid-4'-chloranilide.                            | Brown.                                      |    |
|    | 4:4'-dichloro-2-amino-diphenylether                  | di-(4-methyl-1-hydroxy-2-benzoyl)-dianisidide                                    | Brown.                                      |    |
| 15 | 1-amino-2:5-dimethoxy-4-benzoylaminobenzene          | 2-hydroxyanthracene                                                              | Violet.                                     |    |
|    | 1-amino-2-methoxy-5-methyl-4-benzoylaminobenzene     | 2:3-hydroxynaphthalene-carboxylic acid-anilide                                   | Red.                                        | 15 |
|    | 1-amino-2:5-dimethoxy-4-benzoylaminobenzene          | 3:4-dimethyl-1-hydroxy-benzene-6-carboxylic acid-2'-naphthylamide.               | Brown.                                      |    |
|    | 4:4'-dichloro-2-amino-diphenylether                  | 3-chloro-4-methyl-1-hydroxy-benzene-6-carboxylic acid 2'-methyl-4'-chloranilide. | Brown.                                      |    |
|    | 2-amino-1:5-dimethyl-4-benzoylaminobenzene           | 2:3-hydroxynaphthoic acid-2'-methoxy-anilide                                     | Red.                                        |    |

20 The process permits production of mixed tints by the use of suitable mixtures of parent material, whether of diazo-components or of coupling components, or both together. It can be applied to the most varying textiles, above all to vegetable textiles such as cotton, linen or ramie, further to artificial silk from regenerated cellulose, natural silk and the like.

What we claim is:—

30 1. A process for the production of fast tints on vegetable fiber which comprises printing the fiber with a mixture containing a solid difficultly volatile, diazotizable amine having a melting point not substantially below 60° C., a coupling component, alkali and alkali metal nitrite; then effecting the diazotization of the amine on the fiber without coupling by passing the printed fiber through a dilute aqueous acid solution at a temperature not substantially in excess of 25° C., and then effecting the coupling of the diazotized amine and the coupling component by passing the treated fiber through a dilute aqueous solution of an acid-binding agent.

35 2. A process for the production of fast tints on vegetable fiber which comprises printing the fiber with a mixture containing a solid, difficultly volatile, diazotizable amine having a melting point not substantially below 60° C., an arylide of 2:3-hydroxynaphthoic acid, alkali and alkali metal nitrite; then effecting the diazotization of the amine on the fiber without coupling by passing the printed fiber through a dilute aqueous acid solution at a temperature not substantially in excess of 25° C.; and then effecting the coupling of the diazotized amine and the coupling component by passing the treated fiber through a dilute aqueous solution of an acid-binding agent.

40 3. A process for the production of fast tints on vegetable fiber which comprises printing the fiber with a mixture containing an orthoamino-diphenyl ether having a melting point not substantially below 60° C., an arylide of 2:3-hydroxynaphthoic acid, alkali and alkali metal nitrite; then effecting the diazotization of the amine on the fiber without coupling by passing the printed fiber through a dilute aqueous acid solution at a temperature not substantially in excess of 25° C.; and then effecting the coupling of the diazotized amine and the coupling component by passing the treated fiber through a dilute aqueous solution of an acid-binding agent.

45 4. A process for the production of fast tints on vegetable fiber which comprises printing the fiber with a mixture containing 4:4'-dichloro-2-amino-diphenyl ether, an arylide of 2:3-hydroxynaphthoic acid, alkali and alkali metal nitrite; then effecting the diazotization of the amine on the fiber without coupling by passing the printed fiber through a dilute aqueous acid solution at a temperature not substantially in excess of 25° C.; and then effecting the coupling of the diazotized amine and the coupling component by passing the treated fiber through a dilute aqueous solution of an acid-binding agent.

50 5. A process for the production of fast tints on vegetable fiber which comprises printing the fiber with a mixture containing 4:4'-dichloro-2-amino-diphenyl ether, an ortho-anisidide of 2:3-hydroxynaphthoic acid, alkali and alkali metal nitrite; then effecting the diazotization of the amine on the fiber without coupling by passing the printed fiber through a dilute aqueous acid solution at a temperature not substantially in excess of 25° C.; and then effecting the coupling of the diazotized amine and the coupling component by passing the treated fiber through a dilute aqueous solution of an acid-binding agent.

55 6. A process for the production of fast tints on vegetable fiber which comprises printing the fiber with a mixture containing 4:4'-dichloro-2-amino-diphenyl ether, an ortho-anisidide of 2:3-hydroxynaphthoic acid, alkali and alkali metal nitrite; then effecting the diazotization of the amine on the fiber without coupling by passing the printed fiber through a dilute aqueous acid solution at a temperature not substantially in excess of 25° C.; and then effecting the coupling of the diazotized amine and the coupling component by passing the treated fiber through a dilute aqueous solution of an acid-binding agent.

70 7. A process for the production of fast tints on vegetable fiber which comprises printing the fiber with a mixture containing 4:4'-dichloro-2-amino-diphenyl ether, an ortho-anisidide of 2:3-hydroxynaphthoic acid, alkali and alkali metal nitrite; then effecting the diazotization of the amine on the fiber without coupling by passing the printed fiber through a dilute aqueous acid solution at a temperature not substantially in excess of 25° C.; and then effecting the coupling of the diazotized amine and the coupling component by passing the treated fiber through a dilute aqueous solution of an acid-binding agent.

75 8. A process for the production of fast tints on vegetable fiber which comprises printing the fiber

with a mixture containing a solid, difficultly volatile, diazotizable amine having a melting point not substantially below 60° C. and comprising two aromatic nuclei linked by a N=N bridge, an arylide of 2:3 hydroxynaphthoic acid, alkali and alkali metal nitrite; then effecting the diazotization of the amine on the fiber without coupling by passing the printed fiber through a dilute aqueous acid solution at a temperature not substantially in excess of 25° C.; and then effecting the coupling of the diazotized amine and the coupling component by passing the treated fiber through a dilute aqueous solution of an acid-binding agent.

80 9. A process for the production of fast tints on vegetable fiber which comprises printing the fiber with a mixture containing an orthoamino-diphenyl ether having a melting point not substantially below 60° C., an arylide of 2:3-hydroxynaphthoic acid, alkali and alkali metal nitrite; then effecting the diazotization of the amine on the fiber without coupling by passing the printed fiber through a dilute aqueous acid solution at a temperature not substantially in excess of 25° C.; and then effecting the coupling of the diazotized amine and the coupling component by passing the treated fiber through a dilute aqueous solution of an acid-binding agent.

85 10. A process for the production of fast tints on vegetable fiber which comprises printing the fiber with a mixture containing 4:4'-dichloro-2-amino-diphenyl ether, an arylide of 2:3-hydroxynaphthoic acid, alkali and alkali metal nitrite; then effecting the diazotization of the amine on the fiber without coupling by passing the printed fiber through a dilute aqueous acid solution at a temperature not substantially in excess of 25° C.; and then effecting the coupling of the diazotized amine and the coupling component by passing the treated fiber through a dilute aqueous solution of an acid-binding agent.

90 11. A process for the production of fast tints on vegetable fiber which comprises printing the fiber with a mixture containing 4:4'-dichloro-2-amino-diphenyl ether, an ortho-anisidide of 2:3-hydroxynaphthoic acid, alkali and alkali metal nitrite; then effecting the diazotization of the amine on the fiber without coupling by passing the printed fiber through a dilute aqueous acid solution at a temperature not substantially in excess of 25° C.; and then effecting the coupling of the diazotized amine and the coupling component by passing the treated fiber through a dilute aqueous solution of an acid-binding agent.

95 12. A process for the production of fast tints on vegetable fiber which comprises printing the fiber

- vegetable fiber which comprises printing the fiber with a mixture containing a mono-acidylated-1:4-diaminobenzene having a melting point not substantially below 60° C., an arylide of 2:3-hydroxynaphthoic acid, alkali and alkali metal nitrite; then effecting the diazotization of the amine on the fiber without coupling by passing the printed fiber through a dilute aqueous acid solution at a temperature not substantially in excess of 25° C.; and then effecting the coupling of the diazotized amine and the coupling component by passing the treated fiber through a dilute aqueous solution of an acid-binding agent.
9. A process for the production of fast tints on vegetable fiber which comprises printing the fiber with a mixture containing a mono-acidylated-1:4-diamino - 2:5 - diethoxy-benzene compound whose acyl radical contains a benzene nucleus having a melting point not substantially below 60° C., an arylide of 2:3-hydroxynaphthoic acid, alkali and alkali metal nitrite; then effecting the diazotization of the amine on the fiber without coupling by passing the printed fiber through a dilute aqueous acid solution at a temperature not substantially in excess of 25° C.; and then effecting the coupling of the diazotized amine and the coupling component by passing the treated fiber through a dilute aqueous solution of an acid-binding agent.
10. A process for the production of fast tints on vegetable fiber which comprises printing the fiber with a mixture containing a mono-phenoxo-  
acetyl - 1:4 - diamino - 2:5 - diethoxy-benzene, an arylide of 2:3-hydroxynaphthoic acid, alkali and alkali metal nitrite; then effecting the diazotization of the amine on the fiber without coupling by passing the printed fiber through a dilute aqueous acid solution at a temperature not substantially in excess of 25° C.; and then effecting the coupling of the diazotized amine and the coupling component by passing the treated fiber through a dilute aqueous solution of an acid-binding agent.
11. A process for the production of fast tints on vegetable fiber which comprises printing the fiber with a mixture containing 4:2'-methyl-  
phenoxyacetylamino-1-amino-2:5-diethoxy benzene, the m-chloranilide of 2:3-hydroxy-naphthoic acid, alkali and alkali metal nitrite; then effecting the diazotization of the amine on the fiber without coupling by passing the printed fiber through a dilute aqueous acid solution at a temperature not substantially in excess of 25° C.; and then effecting the coupling of the diazotized amine and the coupling component by passing the treated fiber through a dilute aqueous solution of an acid-binding agent.
12. A process for the production of fast tints on vegetable fiber which comprises printing the fiber with a mixture containing a monoamino-monoazo compound having a melting point not substantially below 60° C., an arylide of 2:3-hydroxynaphthoic acid, alkali and alkali metal nitrite; then effecting the diazotization of the amino on the fiber without coupling bypassing the printed fiber through a dilute aqueous acid solution at a temperature not substantially in excess of 25° C.; and then effecting the coupling of the diazotized amine and the coupling component by passing the treated fiber through a dilute aqueous solution of an acid-binding agent.
13. A process for the production of fast tints on vegetable fiber which comprises printing the fiber with a mixture containing benzene-azo-orthoanisidine, an arylide of 2:3-hydroxynaphthoic acid, alkali and alkali metal nitrite; then effecting the diazotization of the amine on the fiber without coupling by passing the printed fiber through a dilute aqueous acid solution at a temperature not substantially in excess of 25° C.; and then effecting the coupling of the diazotized amine and the coupling component by passing the treated fiber through a dilute aqueous solution of an acid-binding agent.
14. A process for the production of fast tints on vegetable fiber which comprises printing the fiber with a mixture containing benzene-azo-orthoanisidine, an  $\alpha$ -naphthalide of 2:3-hydroxynaphthoic acid, alkali and alkali metal nitrite; then effecting the diazotization of the amine on the fiber without coupling by passing the printed fiber through a dilute aqueous acid solution at a temperature not substantially in excess of 25° C.; and then effecting the coupling of the diazotized amine and the coupling component by passing the treated fiber through a dilute aqueous solution of an acid-binding agent.

ENRICO POOL.

GÉRALD BONHÔTE.

CARL APOTHEKER. 50